

March 25, 1958

E. H. COLLINS ET AL

2,828,081

SEPARATION OF CORK FROM THE BARKS OF TREES

Filed Nov. 19, 1956



ERNEST HOBART COLLINS AND  
EDWARD MURRAY WILLISTON  
INVENTORS

BY

*Leslie G. Waller*  
ATTORNEY

2,828,081

## SEPARATION OF CORK FROM THE BARKS OF TREES

Ernest Hobart Collins, Kelso, and Edward Murray Williston, Longview, Wash., assignors to Weyerhaeuser Timber Company, Tacoma, Wash., a corporation of Washington

Application November 19, 1956, Serial No. 623,233

7 Claims. (Cl. 241—24)

This invention relates to a method for separating from the barks of trees a cork fraction of high yield and purity cork in commercial size to be used as a raw material for structural elements, for insulation, and as a source of chemicals.

The barks of the Douglas fir, the white fir, the ponderosa pine, the western hemlock and other species of trees contain substantial amounts of material called cork, because of its resemblance to the major constituent of the bark of the cork oak. Pieces of bark from separate trees show a wide variation of relative amounts of cork and phloem (largely a mixture of parenchyma tissue and frequently bast fibers or stone cells), grading from pieces consisting almost entirely of phloem and having but thin layers of cork, to those consisting of large masses of cork or phelloiderm with small islands of phloem existing in the cork. The relative amounts of these constituents of bark apparently are affected by such factors as the species of the tree, age, the conditions of growth and the position of the bark on the tree. The bark of the Douglas fir, for example, contains from about 5% to about 50% cork, while that of the white fir contains from about 5% to about 60% cork. This cork component occurs in layers ranging in thickness from the barely visible of about  $\frac{1}{2}$  inch to  $1\frac{1}{2}$  inches with the great bulk occurring in layers ranging from about  $\frac{1}{8}$  to  $\frac{1}{2}$  inch in thickness.

Due to the method of cork formation and the presence of phloem tissue in substantial quantities, and since all of the bark components are intimately commingled and tightly adherent to one another, it is difficult to separate cork of high purity quality and high yield from the barks of trees such as Douglas fir and the white fir.

Past attempts to separate bark components have made use of various comminuting devices to reduce the particle size of the bark followed by various methods for separating or classifying solid material such as screening.

Mere comminution of bark does not result in a clean cut separation of the cork. Rather in the case of Douglas fir bark it results in the formation of a mixture of some small trapezoidal cork particles, a substantial proportion of bast fibers derived from the sclerenchyma tissue, a substantial proportion of fine particles or powder derived from the parenchyma tissue, and a large proportion of aggregates of cork particles and fibers encrusted with or bound together with the parenchyma tissue.

Because the bark mixture contains cork particles, cork aggregate particles, and bark fiber particles of overlapping sizes and weights, the conventional methods of simple screening or air separation are not successfully applicable for the separation of high purity cork in substantial yields.

Also, since a substantial proportion of phloem is tightly adherent to the cork aggregates or appears as islands in the cork particles, screening and air separation techniques still do not produce a high purity cork product

2

even if they are successful in separating the cork and cork aggregates from the fibers and bark powder.

Attempts to produce a high purity cork by a repetition of the steps for comminuting and separating have the disadvantages of drastically reducing the particle size of the cork and at the same time decreasing the cork yield.

It is an object of the present invention to provide a method of separating a high purity cork fraction from the barks of trees.

10 Another object of the present invention is to separate a high purity cork fraction in substantial yields from the barks of trees.

15 It is a further object to separate a high purity cork fraction from the barks of trees in substantial yields and in a relatively large particle size suitable for use in structural materials, insulation products, and as a source of chemicals.

Generally stated, the presently described process comprises reducing bark having a moisture content of 30%

20 to 80% by weight to the form of small pieces having maximum cross-sectional dimensions of less than about  $\frac{1}{2}$  inch. The bark pieces are then dried to a moisture content in the range of between about 6% to 25%. Preferably, the moisture content should be adjusted to

25 a range of from 10% to 12%. The dried bark is then separated into a relatively large particle size cork-rich fraction and a small particle size non-cork fraction. The cork-rich fraction is then passed through a differential speed roller mill which through controlled shearing action

30 breaks up the cork aggregates and removes the tightly adhering phloem without substantially reducing the cork particle size. The product leaving the roller mill is separated to remove a large particle fraction of substantially pure cork. Although this cork fraction has many commercial uses it is preferred to pass the cork through the roller mill a second time with a subsequent separation to

35 further refine the fraction. If essentially pure cork is desired the large particle fraction from the last separation is given a light rod milling and further separation again with the retained material being substantially pure cork of a relatively large particle size.

It will be apparent from the above that a novel principle of the invention resides in the removal of phloem tissue from the cork particles by means of a shear action which does not reduce appreciably the particle size, as contrasted to the pulverizing, grinding methods of previous processes, thus giving a high yield as well as a substantially pure cork.

Furthermore, by minimizing any crushing action, 50 while emphasizing a shearing action, the low apparent density and natural resilience of the cork particle is largely retained as compared to an increase and decrease respectively in these characteristics when using the impacting means of prior methods.

55 It is important that the moisture content be controlled during the passage through the roller mill and subsequent steps. In the range of between about 6% and about 25% by weight much of the moisture is contained in the cork cell particles. In part, because of their relatively high moisture content, the cork particles are

60 resistant to the action of a differential speed roller mill whereas the non-fibrous phloem tissue is relatively dry and brittle and particularly susceptible to shearing stresses. If the moisture content is reduced below about 6% by weight the cork particles become dessicated and hard and tend to pulverize along with the phloem material and the overall large particle size cork yield is drastically reduced.

70 Control of the moisture content in the production of cork from the barks of trees is of still further importance

when considered from the standpoint of the properties of the cork product. When the moisture content of the bark treated is not maintained during the rolling and separating operation at a level sufficiently high to insure that the cork is moist, the cork cells, which are originally turgid, collapse into hard, horny particles from which the resiliency customarily associated with cork is almost completely absent. Since this valuable property may be restored to the dried cork cells only with great difficulty, if at all, over-drying results in destroying the usefulness of the cork product for many applications.

As has been indicated above, the method of this invention may be applied to the bark of any tree containing substantial amounts of cork. It also may be applied to cork rich fractions of bark. Because of their high content of cork and availability, it is particularly applicable to the recovery of cork from the barks of the Douglas fir, the white fir and other commercial coniferous species.

The particular objects and advantages of the invention are described in more detail in the following example and illustrated by reference to the single figure of the drawing which is a flow chart showing the passage of bark through a series of typical processing steps.

#### Procedure

Two separate samples of Douglas fir bark were selected having an original cork content of 44.7% and 24.9% by weight and designated A and B, respectively, in the table following. The samples were processed according to the method as diagrammed by the flow chart of the figure. The whole bark was comminuted by passing through a grinder, specifically a Jacobsen pulverizer, driven by a  $\frac{3}{4}$  H. P. motor at a no-load speed of 4300 R. P. M. and having  $\frac{1}{4}$  in. screen. After passing through the grinder the moisture content of the bark was 35-40%. The small pieces of bark were dried to a moisture content of 10-12% in a non-circulating oven at approximately 180° F. and screened on a Denver-Dillon vibrating screen set with a screen inclination of about 25° to the horizontal. The plus 30 mesh fraction is retained in the process and passed through a roller mill having machined steel rolls, 12" in length and 5.8" in diameter, mounted in a horizontal plane with a static roll nip clearance set at 0.007 inch. The rolls are geared for a 1 to 1.3 differential speed. In these experiments the actual speeds of the rollers were 20 and 26 R. P. M. The bark fraction was fed directly into the nip, along the length of the rolls and doctor blades were used to prevent the bark material from adhering to the rolls and recycling through the nip. The roller mill is water cooled to prevent sheeting caused by exudation of waxes from the cork particles. The bark is again separated by passing over the vibrating screen and the plus 30 mesh fraction is passed again through the roller mill. The vibrating screen set is used to separate the bark material and the plus 30 mesh fraction is further refined in a rod mill having a cylindrical cavity, 15" long and  $6\frac{1}{2}$ " in diameter, rotating at 50 R. P. M. This was a batchwise operation using 300 grams of bark material and approximately 29,000 grams of steel rods consisting of 20 ( $\frac{3}{4}$ " by  $13\frac{1}{2}$ ") rods and 20 ( $\frac{3}{8}$ " by  $13\frac{1}{2}$ ") rods. The bark material was screened and a plus 28 mesh fraction became the final cork product.

The screen sizes are based on the Tyler standard screen scale with a 28 mesh screen having an opening of .0232 inch which for many commercial uses of cork is a minimum particle size.

The following table shows the cork yield and purity of product for the same particle size range after each step of the process. By way of comparison, yield and purity data are included under C for a typical analysis of a product resulting from a method wherein a roller mill is omitted and all refining is done in a ball mill after the initial comminuting and screening.

| 5                                        |  | Percent of Starting Cork Material Retained |       |       | Percent of Cork in Product Retained |       |       |
|------------------------------------------|--|--------------------------------------------|-------|-------|-------------------------------------|-------|-------|
|                                          |  | A                                          | B     | C     | A                                   | B     | C     |
| Original                                 |  | 100                                        | 100   | 100   | 44.7                                | 24.9  | 34.6  |
| Comminuted and Screened                  |  | 96                                         | 91.4  | ----- | 51.8                                | 30.1  | ----- |
| Sheared in Roller Mill and Screened      |  | 89.7                                       | 78.3  | ----- | 64.7                                | 48.3  | ----- |
| 10 2nd Roller Mill and Screened          |  | 85.4                                       | 70.5  | ----- | 77.5                                | 64.0  | ----- |
| Rolled and beat in Rod Mill and Screened |  | 76.2                                       | 40.9  | ----- | 88.2                                | 89.7  | ----- |
| Ball Mill, no Roller Mill                |  | -----                                      | ----- | 15.0  | -----                               | ----- | 65.0  |
| Ball Mill, no Roller Mill                |  | -----                                      | ----- | 5-7.0 | -----                               | ----- | 89.0  |

15 (Cork content analyses were made by a technique which consists of immersing the sample to be tested in a solution of carbon tetrachloride and benzene having a specific gravity of 1.38. The cork is determined as that portion of the bark material which floats on the solution.)

20 It is readily apparent by reference to the above table that for a product of similar particle size (+28 mesh) and similar cork content (approximately 65%) the use of a differential speed roller mill provides a means of increasing the cork yield approximately 4.5 to 6 times that of previous methods depending on the cork content of the starting bark material.

25 The value of the method of this invention assumes even greater importance when we observe from the above table that for a similar particle size of a bark product of approximately 90% cork content the yield by this method is in the range from about 6 to 10 times that of a pulverizing, impacting method.

30 Although not wishing to be bound by any theory, it is believed that the method of this invention recognizes the inherent differences in the elastic and friable characteristics of the various components of bark under controlled moisture contents and, at the same time, that the nature of the bond between them is such that the application of a shear rather than an impact stress provides the most efficient and effective means of rupturing such bond.

35 No limitation is intended by reference to a particular type of apparatus for practicing the method of the invention, the same being limited only by the scope of the appended claims. In particular, applicants do not wish to be limited to the specific apparatus referred to for performing the comminuting, grinding, and shearing steps, nor do applicants wish to be limited to separation by screening or to specific sizes of screen openings. References in the specification to particular apparatus and screen openings are made by way of illustration only, to describe a preferred manner of carrying out the steps of the method in a continuous process best suited for a production plant. Other apparatus for grinding and comminuting, and for applying shearing stresses may be devised by those skilled in the art and some variance may be made in the screening apparatus. Alternative means of separation, such as a winnower or a centrifuge, may be used by properly coordinating the variables mentioned in the specification. All such modifications and variations are included in the invention.

40 Having now described our invention and in what manner the same may be used, what we claim as new and desire to protect by Letters Patent is:

45 1. The method of treating Douglas fir bark and mixtures of components thereof for the production of a substantially pure cork fraction which comprises comminuting the bark having a moisture content of from 30 to 80% by weight to produce small particles having maximum cross-sectional dimensions of less than  $\frac{1}{2}$  inch; drying the bark particles to a moisture content of from 6 to 25%; separating the bark particles into a large particle size cork-rich fraction and a small particle size non-cork fraction; shearing the particles of the cork-rich fraction to break up the cork aggregates and remove the phloem; separating a second large particle fraction of

cork; shearing the said second cork fraction to further refine it; separating a third large particle fraction of cork; lightly rolling and beating the said third cork fraction; and separating a final large particle fraction of essentially pure cork.

2. The method of claim 1 wherein the shearing steps are performed by passing the cork fractions through a differential speed roller mill.

3. The method of claim 1 wherein the rolling and beating step is performed by passing the cork fraction through a rod mill.

4. The method of treating Douglas fir bark and mixtures of components thereof for the production of a substantially pure cork fraction which comprises comminuting the bark having a moisture content of from 30 to 80% by weight to produce small particles having maximum cross-sectional dimensions of less than  $\frac{1}{2}$  inch; drying the bark particles to a moisture content of from 6 to 25%; separating the bark particles into a large particle size cork-rich fraction and a small particle size non-cork fraction; shearing the particles of the cork-rich fraction to break up the cork aggregates and remove the phloem; separating a second large particle fraction of cork; shearing the said second cork fraction to further refine it; and separating a third large particle fraction of cork.

5. The method of treating Douglas fir bark and mixtures of components thereof for the production of a substantially pure cork fraction which comprises comminuting the bark having a moisture content of from 30 to 80% by weight to produce small particles having maximum cross-sectional dimensions of less than  $\frac{1}{2}$  inch; drying the bark particles to a moisture content of from 6 to 25%; separating the bark particles into a large particle size cork-rich fraction and a small particle size non-cork fraction; shearing the particles of the cork-rich fraction to break up the cork aggregates and remove the phloem; separating a second large particle fraction of cork; lightly rolling and beating the said second cork fraction; and separating a final large particle fraction of essentially pure cork.

6. The method of treating Douglas fir bark and mix-

tures of components thereof for the production of a substantially pure cork fraction which comprises comminuting the bark having a moisture content of from 30 to 80% by weight to produce small particles having maximum cross-sectional dimensions of less than  $\frac{1}{2}$  inch; drying the bark particles to a moisture content of from 6 to 25%; separating the bark particles into a large particle size cork-rich fraction and a small particle size non-cork fraction; shearing the particles of the cork-rich fraction to break up the cork aggregates and remove the phloem; separating a second large particle fraction of cork; shearing the said second cork fraction to further refine it; and separating a third large particle fraction of cork.

15 7. The method of treating Douglas fir bark and mixtures of components thereof for the production of a substantially pure cork fraction which comprises comminuting the bark having a moisture content of from 30 to 80% by weight to produce small particles having maximum cross-sectional dimensions of less than  $\frac{1}{2}$  inch; drying the bark particles to a moisture content of from 10 to 12%; separating the bark particles into a large particle size cork-rich fraction and a small particle size non-cork fraction; shearing the particles of the cork-rich fraction 20 to break up the cork aggregates and remove the phloem; separating a second large particle fraction of cork; shearing the said second cork fraction to further refine it; separating a third large particle fraction of cork; lightly 25 rolling and beating the said third cork fraction; and separating a final large particle fraction of essentially pure cork.

#### References Cited in the file of this patent

#### UNITED STATES PATENTS

|    |           |                |               |
|----|-----------|----------------|---------------|
| 35 | 2,437,672 | Anway          | Mar. 16, 1948 |
|    | 2,444,929 | Hatch          | July 13, 1948 |
|    | 2,446,551 | Pauley         | Aug. 10, 1948 |
|    | 2,627,375 | Grondal et al. | Feb. 3, 1953  |